

# United States Patent Office

3,058,826

Patented Oct. 16, 1962

1

3,058,826

## PHOTOGRAPHIC ELEMENTS EXHIBITING REDUCED HAZE AND METHOD FOR PREPARATION

Beat Meerkamper, Red Bank, and Jacob Quentin Umbberger, Holmdel, N.J., assignors to E. I. du Pont de Nemours and Company, Wilmington, Del., a corporation of Delaware

No Drawing. Filed Dec. 11, 1959, Ser. No. 858,865

5 Claims. (Cl. 96—67)

This invention relates to photographic elements comprising a support coated with a gelatino-silver halide emulsion containing an agent for increasing the covering power of the developed silver. This invention more particularly relates to a method of improving such photographic elements by increasing the speed and improving the clarity and reducing the turbidity of the processed emulsion layers containing poly-N-vinylactams as covering power increasing agents.

The use of poly-N-vinylactam covering power increasing agents in gelatino-silver halide emulsions is disclosed and claimed in assignee's copending application of Overman et al., U.S. Ser. No. 748,605 filed July 15, 1958, now abandoned. As shown in that application, the presence of the compounds disclosed therein increases the efficiency of the silver halide in the system. This efficiency manifests itself by increases in effective speed, contrast or gamma. Such increases in silver halide efficiency are much to be desired in certain types of photographic elements such as films for radiological use and films for use in the graphic arts field.

However, the use of such agents in gelatino-silver halide emulsion systems produces photographic emulsions which show a tendency toward turbidity or haziness in the coated and processed emulsion layer which is undesirable and in turn causes undesirable effects on definition.

The use of gelatin antiabrasion coatings over gelatino-silver halide emulsion layers is very old in the art and such layers are generally coated in such a manner as to give a dry coating weight of not more than 10 milligrams per square decimeter. It is known that heavy gelatin abrasion layers, e.g., up to 10 milligrams per square decimeter, are necessary in the case of X-ray emulsions because of the greater susceptibility of such emulsions to abrasion.

Further, it is known to use poly-N-vinylactams as the sole binder for photographic silver halide emulsions. It is also known to add polyvinyl pyrrolidone and copolymers thereof to gelatino-silver halide emulsions to overcome yellow fog. In addition it is known to add polyvinyl pyrrolidone to gelatino-silver halide emulsions or to image receptive layers for use in the so-called inverse transfer process. In this latter case it is used in quantities up to 40 parts or more per 100 parts of total binder to produce a turbid or non-homogeneous layer when the emulsion is coated and dried. The non-homogeneity is for the purpose of lowering the cohesiveness of the emulsion layer and the receptive layer during the inverse transfer process. X-ray emulsions can also be used in this inverse transfer process. However, no art is known where gelatin layers so heavy as to be outside the category of antiabrasion layers have been coated over emulsions containing covering power increasing agents.

An object of this invention is to provide photographic elements which have reduced haze and methods for their production. A further object is to provide such elements, which have reduced haze despite the use in the photographic emulsions of poly-N-vinylactam covering power increasing agents, and methods for production. A still further object is to provide such elements which result in improved sensitometric characteristics and

2

methods for their production. Other objects will appear hereinafter.

These and other objects have been quite unexpectedly accomplished by the following invention which comprises a method for producing photographic elements having reduced haze which comprises coating a macromolecular polymeric base support with a layer of photographic emulsion containing poly-N-vinylactam covering power increasing agent, and coating a heavy layer of gelatin thereover in sufficient quantity to reduce the haze in said element. The heavy gelatin layers not only reduce haze to acceptable levels, but, as a consequence, such layers increase the resolution of the resulting photographic elements. Most surprisingly, the heavy gelatin overcoatings produce increased photographic speed.

In general, it has been found that a coating weight of from 20 to 40 milligrams of gelatin based on dry weight per square decimeter is quite efficacious in producing the advantageous effects of the invention. The gelatin solutions for coating the heavy overcoating layers may vary in concentration over a wide range but, in general, a concentration of from 3 to 10% will be found to be suitable. In addition, the heavy overcoating layers provide an improved degree of gloss, possibly associated with the emulsion speed increase, to the surface of the coated element when viewed by reflected light. This becomes reasonable when it is realized that 20 mg./dm.<sup>2</sup> of gelatin is equivalent in thickness to 1.6 microns of AGBr, the average particle size of high-speed emulsions such as are employed in medical X-ray films. The method of applying the relatively heavy gelatin overcoating is not too critical and the emulsion layer may be overcoated in the wet or dry state. There is, however, a somewhat greater reduction in haze when the emulsion is overcoated wet. This is of considerable importance because in the manufacture of overcoated photographic elements as it is now sometimes carried out, antiabrasion layers are applied successively to freshly coated emulsion layers while the latter are still wet. The haziness in the dried emulsion layers coated from emulsions containing the covering power increasing agents noted above is of course, caused by light scattering in the emulsion and/or at the emulsion/air interface. Therefore, the haze may be measured by determining the amount of scattered light when passing through any particular film from which the silver halide has been removed by fixation. It is preferable to make the haze determination on unexposed and undeveloped films since the fog/silver deposits also scatter light. The haze measurements in the following examples were made on undeveloped samples and are therefore independent of the fog level. The measurements were made on a "Lumetron" Model 402E photoelectric colorimeter sold by the Photovolt Corporation, 95 Madison Avenue, New York 60, New York.

55 As a means of interpreting the figures derived in measuring the films of the examples, the following standard values for haze are given which are relative numbers indicating the fraction of light that is scattered through the film:

60 0-6 clear  
6-15 detectable (not noticeable on light box viewing)  
15-40 transparent haze  
40+ milky or turbid

65 The invention will now be illustrated in and by the following examples.

### EXAMPLE I

A high speed gelatino-silver iodobromide emulsion was 70 made containing 54% silver halide which was approximately 2 mole percent iodide and 98 mole percent bromide, and containing 34% gelatin based on total solids.

It was digested with an organic sulfur compound and gold chloride. After digestion, 36.4 grams per mole of silver halide of poly-N-vinyl-2-pyrrolidone (PVP) having a molecular weight of approximately 45,000 was added to give 12% of PVP based on total solids. The resulting emulsion was coated on two strips of conventionally subbed cellulose acetate film base in an amount to give a dry coating weight of 100 milligrams of silver halide per square decimeter. The coated films were then dried in a conventional manner. One coated film was overcoated with a 3% aqueous gelatin solution containing 0.02 milligram of chrome alum and 0.03 milligram of dimethylol urea per milligram of gelatin. The dry coating weight of the overcoating was 10 milligrams per square decimeter. The other coated film was over-

5 10 15

#### 4 EXAMPLE II

A gelatino-silver iodobromide emulsion was made as described in Example I and sixteen emulsion coatings were made, eight of which were overcoated to give a dry coating weight of 10 mg./dm.<sup>2</sup> from a 3% aqueous gelatin solution and eight others were overcoated to give a dry coating weight of 30 mg./dm.<sup>2</sup> from a 9% aqueous gelatin solution. The aqueous gelatin overcoating solutions contained varying amounts of chrome alum and dimethylolurea hardening agents as indicated in the table. Haze, was measured on the fixed, washed and dried films. Sensitometric data were obtained on films which had been exposed to a low intensity X-ray exposure and processed as described in Example I. The results are shown in the following table.

TABLE I

| Coating Number | Hardener                                     |                                   |                                       | Sensitometry |          |                  |       |     |
|----------------|----------------------------------------------|-----------------------------------|---------------------------------------|--------------|----------|------------------|-------|-----|
|                | Coating Weight Gelatin, mg./dm. <sup>2</sup> | Chrome Alum, mg./dm. <sup>2</sup> | Dimethylol Urea, mg./dm. <sup>2</sup> | Over-Coated  | Haze Dry | Speed (Relative) | Gamma | Fog |
| 1              | 10                                           | 0.2                               | None                                  | Wet-----     | 33       | 159              | 2.7   | .07 |
| 2              | 10                                           | 0.2                               | None                                  | Dry-----     | 29       | 142              | 2.5   | .14 |
| 3              | 10                                           | 0.2                               | 0.3                                   | Wet-----     | 30       | 154              | 2.2   | .07 |
| 4              | 10                                           | 0.2                               | 0.3                                   | Dry-----     | 29       | 156              | 2.1   | .11 |
| 5              | 10                                           | None                              | 0.3                                   | Wet-----     | 27       | 152              | 2.1   | .05 |
| 6              | 10                                           | None                              | 0.3                                   | Dry-----     | 25       | 127              | 2.2   | .12 |
| 7              | 10                                           | None                              | None                                  | Wet-----     | 26       | 164              | 2.3   | .07 |
| 8              | 10                                           | None                              | None                                  | Dry-----     | 28       | 143              | 2.3   | .12 |
| 9              | 30                                           | None                              | None                                  | Wet-----     | 11       | 177              | 2.1   | .07 |
| 10             | 30                                           | None                              | None                                  | Dry-----     | 13       | 150              | 2.3   | .15 |
| 11             | 30                                           | None                              | 0.3                                   | Wet-----     | 13       | 177              | 2.0   | .06 |
| 12             | 30                                           | None                              | 0.3                                   | Dry-----     | 13       | 153              | 2.1   | .17 |
| 13             | 30                                           | 0.2                               | 0.3                                   | Wet-----     | 11       | 194              | 2.1   | .06 |
| 14             | 30                                           | 0.2                               | 0.3                                   | Dry-----     | 11       | 152              | 2.2   | .14 |
| 15             | 30                                           | 0.2                               | None                                  | Wet-----     | 11       | 174              | 2.2   | .07 |
| 16             | 30                                           | 0.2                               | None                                  | Dry-----     | 12       | 142              | 2.3   | .17 |

coated with a 9% aqueous gelatin solution containing about 0.007 milligram of chrome alum and about 0.01 milligram of dimethylol urea per milligram of gelatin. The dry coating weight was 30 milligrams per square decimeter. These two films were dried in a conventional manner. The two films were exposed to low intensity X-rays in the presence of an intensifying screen through an aluminum square root of two step-wedge according to a procedure based on the American Standard Method for the Sensitometry of Medical X-Ray Films—Ph 2.9—1956. The exposed coatings were developed for 5 minutes in a developer having the following composition:

|                                     | Grams |
|-------------------------------------|-------|
| N-methyl-p-aminophenol hydrosulfate | 3     |
| Sodium sulfite (anhydrous)          | 50    |
| Hydroquinone                        | 9     |
| Potassium carbonate (anhydrous)     | 50    |
| Potassium bromide                   | 4.5   |
| Water to make 1 liter.              |       |

The coatings were then fixed, washed and dried in a conventional manner. Results of sensitometric tests for speed, gamma and fog for all tests are given below. Speed is given in terms of reciprocal of exposure at a density of 0.7. Haze measurements are relative numbers described above.

## Law Intensity Exposure

| Coating                 | Speed (Relative) | Gamma | Fog | Dry Haze |
|-------------------------|------------------|-------|-----|----------|
| 10 mg./dm. <sup>2</sup> | 390              | 3.08  | .08 | 19.8     |
| 30 mg./dm. <sup>2</sup> | 410              | 3.80  | .07 | 8.0      |

It will be noted that there was a significant reduction in haze where the heavy gelatin overcoating was used and also that the sensitometric characteristics were either unaffected or improved.

45 50 55 60 70

A gelatino-silver iodobromide emulsion was made as described in Example I and two coatings were made having a dry coating weight of 100 milligrams of silver halide per square decimeter. The coated films were dried in the conventional manner and one coating was used as a control and not treated further. One coating was overcoated with a 3% aqueous gelatin solution containing 18 milligrams of formaldehyde per gram of gelatin of give a dry coating weight of 10 milligrams per square decimeter. The other coating was overcoated with a 9% aqueous gelatin solution containing 18 milligrams of formaldehyde per gram of gelatin to give a dry coating weight of 30 milligrams per square decimeter. Haze was measured on the fixed, washed and dried films. Sensitometric data were obtained on films which had been exposed to a low intensity X-ray exposure and processed as described in Example I. The results are shown in the following table.

| Coating | Abrasion Coating, Weight | Haze | Speed (Relative) | Sensitometry |     |
|---------|--------------------------|------|------------------|--------------|-----|
|         |                          |      |                  | Gamma        | Fog |
| 2       | 10                       | 12   | 156              | 2.0          | .08 |
| 3       | 30                       | 8    | 152              | 1.85         | .07 |

It will be seen that the use of heavy gelatin abrasion overcoating decreases the haze to a considerable degree and that formaldehyde hardening does not interfere with the effect. Sensitometric characteristics were also not detrimentally affected.

The invention is not limited to photographic gelatino-silver halide emulsions of the silver iodobromide type. The invention may be applied to other gelatino-silver halide emulsions, e.g., gelatino-silver bromochloride emulsions of the lithographic type. The invention is also not limited to overcoating gelatino-silver halide emulsions containing poly-N-vinyl-2-pyrrolidone as the covering power increasing agent. Silver halide emulsions containing poly-N-vinylcaprolactam, poly-N-vinyl-5-methyl-2-pyrrolidone and poly-N-vinylpiperidone may also be beneficially aided by the heavy gelatin overcoatings of the invention. The invention is particularly efficacious with photographic emulsions whose grain size is relatively large. The emulsions to be overcoated may contain any of the well known optical sensitizing dyes as well as non-optical sensitizers such as sulfur sensitizers containing labile sulfur, e.g., allyl isothiocyanate, allyl diethyl thiourea, phenyl isothiocyanate and sodium thiosulfate; the polyoxyalkylene ethers disclosed in Blake et al., U.S. Patent 2,400,532 and the polyglycols disclosed in Blake et al., U.S. Patent 2,423,549. Other non-optical sensitizers such as amines as taught by Staud et al., U.S. Patent 1,925,508 and metal salts as taught by Baldsiefen U.S. Patent 2,540,085 and Baldsiefen et al., U.S. Patent 2,540,086 may also be used. Antifoggants, e.g., benzotriazole, triazaindenes and the phenolic antifoggants disclosed in assignee's copending application, Forsgard, U.S. application Serial No. 757,460 filed August 27, 1958, may be used. Any of the usual film supports of macromolecular polymeric materials may be used such as cellulose esters, e.g., cellulose triacetate, cellulose acetate/butyrate; superpolymers, e.g., polystyrene, poly (vinyl chloride or vinyl acetate); polyvinyl acetals, e.g., formal and acetal; polyamides, e.g., polyhexamethylene adipamide, and polyesters, e.g., polyethylene terephthalate. The vinylidene chloride copolymer-coated oriented polyester films of Alles et al., U.S. Patent 2,627,088 are especially suitable.

The novel overcoating may be applied by any suitable means such as skim coating over the undried emulsion layer as taught by Daily, U.S. Patent 1,699,349 and Dixon, U.S. Patent 1,892,484 or by the apparatus disclosed in assignee's copending applications of Brandsma et al., Serial No. 849,376, filed October 28, 1959 and Beck, U.S. application Serial No. 506,458, filed May 6, 1955.

An advantage of the invention is that the heavy gelatin overcoating provides a simple method of taking full advantage of the new discovery of using covering power increasing agents to improve maximum density, contrast and effective speed of gelatino-silver halide emulsions.

Another advantage of the invention is that the heavy gelatin overcoatings can be applied by the ordinary technician with conventional apparatus. Since aqueous gelatin solutions are used, no volatile solvents are involved

necessitating the use of solvent recovery systems. Conventional coating and drying equipment can be used to practice the invention.

What is claimed is:

- 5 1. A method for producing photographic elements having reduced haze which comprises coating a macromolecular polymeric base support with a layer of photographic gelatino-silver halide emulsion containing poly-N-vinylactam silver covering power increasing agent and coating a layer of gelatin thereover of from 20 to 40 mg. of gelatin per square decimeter, based on dry weight.
- 10 2. A method for producing photographic elements having reduced haze which comprises coating a macromolecular polymeric base support with a layer of photographic gelatino-silver iodobromide emulsion containing polyvinyl pyrrolidone silver covering power increasing agent and coating a layer of gelatin thereover of from 20 to 40 mg. of gelatin per square decimeter, based on dry weight, said gelatin being applied to said emulsion layer as an aqueous solution of from 3 to 10% gelatin by weight.
- 15 3. Method according to claim 2 wherein said emulsion layer is still wet when the gelatin layer is coated thereover.
- 20 4. A photographic element having reduced haze comprising a macromolecular polymeric base support having coated thereover a photographic emulsion layer containing poly-N-vinylactam silver covering power increasing agent, said emulsion layer having coated thereover an overcoating of gelatin in an amount of from 20 to 40 mg. of gelatin per square decimeter, based on dry weight.
- 25 5. A photographic element having reduced haze comprising a macromolecular polymeric base support having coated thereover a photographic gelatino-silver halide emulsion layer containing polyvinyl pyrrolidone silver covering power increasing agent, said emulsion layer having coated thereover an overcoating of gelatin in an amount of from 20 to 40 mg. of gelatin per square decimeter, based on dry weight.
- 30 35 6. A photographic element having reduced haze comprising a macromolecular polymeric base support having coated thereover a photographic gelatino-silver halide emulsion layer containing polyvinyl pyrrolidone silver covering power increasing agent, said emulsion layer having coated thereover an overcoating of gelatin in an amount of from 20 to 40 mg. of gelatin per square decimeter, based on dry weight.

#### References Cited in the file of this patent

##### UNITED STATES PATENTS

- |           |                    |               |
|-----------|--------------------|---------------|
| 2,415,624 | Brown et al. ----- | Feb. 11, 1947 |
| 2,948,614 | Allen et al. ----- | Aug. 9, 1960  |
| 2,995,444 | Dersch -----       | Aug. 8, 1961  |

##### FOREIGN PATENTS

- |         |                     |               |
|---------|---------------------|---------------|
| 609,826 | Great Britain ----- | Oct. 7, 1947  |
| 687,751 | Great Britain ----- | Feb. 18, 1953 |

##### OTHER REFERENCES

- Glafkides: Photographic Chemistry, vol. I, Fountain Press, London, 1958, page 474,